

# United States Patent [19]

Merz et al.

[11] 3,854,827

[45] Dec. 17, 1974

[54] METAL-TO-CERAMIC LEADTHROUGH

[75] Inventors: Josef Merz, Hamburg, Germany; Johannes Van Esdonk; Joannes Franciscus Maria Janssen, both of Emmasingel, Eindhoven, Netherlands

[73] Assignee: U.S. Philips Corporation, New York, N.Y.

[22] Filed: Nov. 22, 1972

[21] Appl. No.: 308,685

[30] Foreign Application Priority Data

Dec. 1, 1971 Germany..... 2159531

[52] U.S. Cl. .... 403/29

[51] Int. Cl. .... F16b 11/00, C03c 27/02

[58] Field of Search ..... 403/28, 29, 179, 270, 271; 52/759; 65/36, 59; 29/180 NM

[56] References Cited

UNITED STATES PATENTS

2,200,694 5/1940 Gerecke et al. .... 29/180 NM

|           |         |                     |          |
|-----------|---------|---------------------|----------|
| 3,219,753 | 11/1965 | Vassos .....        | 403/28 X |
| 3,278,211 | 10/1966 | Baas et al. ....    | 403/29   |
| 3,370,874 | 2/1968  | Scherer et al. .... | 403/28   |
| 3,385,618 | 5/1968  | Hargis .....        | 403/271  |
| 3,436,109 | 4/1969  | Loose .....         | 52/759   |
| 3,545,950 | 12/1970 | Earl .....          | 65/59    |
| 3,600,017 | 8/1971  | Scherer.....        | 52/759   |

Primary Examiner—Werner H. Schroeder  
Attorney, Agent, or Firm—Frank R. Trifari

[57]

## ABSTRACT

A metal-to-ceramic leadthrough with the use of glass-like material and an aperture having a narrow portion which changes in a step-wise manner into a widened portion, the gap between the conductor and the wall of the narrow portion being filled entirely with glass-like material and the bottom of the wide portion of the aperture being covered with a thin layer of glass-like material which forms a meniscus against the conductor and the inner wall of the wide portion of the aperture.

2 Claims, 1 Drawing Figure



PATENTED DEC 17 1974

3,854,827



**METAL-TO-CERAMIC LEADTHROUGH**

The invention relates to a metal-to-ceramic leadthrough, in particular a liquid-tight or vacuum-tight leadthrough, in which a metal conductor is secured by means of a glass-like material in a ceramic wall having a thickness of more than 2 mm while using an aperture having a stepwise-widened portion. The invention relates in particular to such a leadthrough of a conductor having a coefficient of thermal expansion lower than that of the ceramic portion, for example, a conductor consisting of molybdenum.

Such a leadthrough is known from the U.S. Pat. No. 3,545,950. In this patent the wide portion of the aperture is filled by means of a member consisting of a glass-like material which has a cavity on its upper side. By accurately controlled heating it is achieved that the glasslike material softens in such manner as to adhere to the conductor and to the inner wall of the widened portion of the aperture but without a meniscus being formed against the metal surface and without the gap between the conductor and the inner wall of the narrow portion of the aperture being filled. The glass-like material may thus not become thin-liquid.

It has been found, however, that as a result of such a large accumulation of glass-like material in the wide portion of the aperture, cracks can occur in the glass-like material during cooling after softening said material. This is the case also if a conductor is secured in a wall having a thickness of more than 2 mm by means of a glass-like material while using a narrow aperture having a constant diameter.

It has been found that the said difficulty can be avoided entirely in a metal-to-ceramic leadthrough in which a metal conductor is secured in an aperture of a ceramic wall having a thickness of more than 2 mm by means of glass-like material, which aperture consists of a narrow portion which changes step-wise into a wider portion, it, according to the invention, the quantity of glass-like material is chosen and provided in such manner and is heated to such a high temperature that the glass-like material has entirely filled the gap between the conductor and the inner wall of the narrow portion of the aperture, but has formed a comparatively thin layer on the bottom of the wide portion of the aperture, said thin layer forming a meniscus both against the conductor and against the inner wall of the wide portion of the aperture. The length of the narrow portion of the aperture may preferably be equal to that of the wide portion but must at least be so large that the desired seal is obtained but may at most not exceed approximately 2 mm so as to avoid cracking of the glass-like layer during cooling after melting thereof or afterwards during operation. Since the thin glass-like layer forms a meniscus on the bottom of the wide portion of the aperture against the metal surface and against the inner wall of said portion of the aperture, it has been found that in this case also no cracks are formed while a sufficient mechanical rigidity is obtained. The thickness of the glass-like layer on the bottom of the wide portion of the aperture is from 100 to 1,000  $\mu$ , which layer forms a meniscus towards the edge of the conductor and towards the inner wall of the aperture. The diameter of the wide portion of the aperture is preferably three to four times as large as the diameter of the narrow portion.

The glass-like material preferably has the following composition:

37 percent by weight MnO,

50 percent by weight SiO<sub>2</sub>

13 percent by weight Al<sub>2</sub>O<sub>3</sub>.

Melting is carried out at 1,300°C for 10 minutes. The conductor may consist of molybdenum which is necessary for certain applications.

In metal-to-ceramic joints it is known to use apertures which are widened in a step-wise manner, for example, from the U.S. Pat. No. 3,385,618 in which a metal solder is used which forms a meniscus against the conductor and a thin layer on the bottom of the wide portion. In this case, however, the gap between the conductor and the inner wall of the narrow portion of the aperture must remain free from soldering material so as to be able to compensate for the difference in coefficients in thermal expansion between metal and ceramic. The widened portion of the aperture serves to be able to metallize the whole surface and to be able to remove said metal layer afterwards from the upper surface, the metal layer on the bottom of the widened portion of the aperture being maintained which is necessary to cause the metal solder to flow.

In the U.S. Pat. No. 2,731,578 the widened aperture is provided so as to obtain an insulation path between the metallized surface of the ceramic part and the leadthrough conductor. In British Pat. No. 522,217 the widened portion of the aperture is provided so as to be able to connect any contact members to the leadthrough conductor. When using metallic soldering material, however, the circumstances are quite different from those occurring when a glass-like material is used.

The invention will be described in greater detail with reference to the accompanying drawing, the FIGURE of which shows a metal-to-ceramic leadthrough according to the invention.

Reference numeral 1 in the FIGURE denotes a ceramic wall of 4 mm thickness through which a molybdenum conductor 2 having a diameter of 1.5 mm is passed. The aperture in the wall 1 has a narrow portion 3 having a diameter of 1.6 mm and a widened portion 4 having a diameter of 6 mm. The gap between the conductor 2 and the inner wall of the portion 3 of the aperture is entirely filled with glass-like material 5 of the above-described composition. the bottom of the portion 4 of the aperture is covered with a layer 6 of the glass-like material 5. The thickness of the layer 6 may be from 100 to 1,000  $\mu$ . The layer 6 forms a meniscus 7 both on the metal surface of the leadthrough conductor 2 and on the inner wall 8 of the portion 4 of the aperture. After placing the conductor 2 in the aperture, the suspension is provided on the bottom of the wide portion 4. Melting occurs in a reducing atmosphere at a temperature of 1,300°C for 10 minutes, the layer 6 with the meniscus 7 being formed and the gap between the conductor 2 and the inner wall of the aperture 3 being filled. Since the way of heating is not critical, a ceramic wall having a large number of leadthrough conductors may be heated in a furnace in which all the conductors are sealed simultaneously.

Metal-to-ceramic leadthroughs according to the invention have proved particularly suitable for use in digital light deflection systems which are provided in a ceramic vessel, said vessel being filled with liquid and the leadthrough conductors consisting of molybdenum.

What is claimed is:

1. A metal-to-ceramic leadthrough, comprising: a ceramic wall portion that has a thickness of more than 2

mm and that includes an aperture comprising a narrow portion which changes in a step-wise manner into a wider portion, said narrow portion having a length that is at most about 2 mm; a metal conductor disposed in said aperture and spaced by a gap from the aperture wall; and a body of glass-like material disposed at and entirely filling the gap between the conductor and the inner wall of the narrow portion of the aperture, said body forming a relatively thin layer on the bottom of the wide portion of the aperture and said thin layer

5 forming a meniscus both against the conductor and against the inner wall of the wide portion of the aperture, said conductor consisting of a material having a coefficient of thermal expansion which is lower than that of the ceramic portion.

2. A metal-to-ceramic leadthrough as in claim 1, wherein said conductor material consists essentially of molybdenum.

10

\* \* \* \* \*

15

20

25

30

35

40

45

50

55

60

65

UNITED STATES PATENT OFFICE  
CERTIFICATE OF CORRECTION

Patent No. 3,854,827

Dated December 17, 1974

Inventor(s) JOSEF MERZ ET AL

It is certified that error appears in the above-identified patent and that said Letters Patent are hereby corrected as shown below:

On the title page, Section [30] change "215931"

to --P.215931. 3--.

Signed and sealed this 18th day of February 1975.

(SEAL)

Attest:

RUTH C. MASON  
Attesting Officer

C. MARSHALL DANN  
Commissioner of Patents  
and Trademarks